



US006436480B1

(12) **United States Patent**  
**Upadhyा**

(10) **Patent No.:** **US 6,436,480 B1**  
(b4) **Date of Patent:** **\*Aug. 20, 2002**

(54) **THERMAL SPRAY FORMING OF A COMPOSITE MATERIAL HAVING A PARTICLE-REINFORCED MATRIX**

(75) Inventor: **Kamleshwar Upadhyā**, Quartz Hill, CA (US)

(73) Assignee: **Plasma Technology, Inc.**, Torrance, CA (US)

(\*) Notice: Subject to any disclaimer, the term of this patent is extended or adjusted under 35 U.S.C. 154(b) by 0 days.

This patent is subject to a terminal disclaimer.

(21) Appl. No.: **09/607,132**

(22) Filed: **Jun. 29, 2000**

**Related U.S. Application Data**

(63) Continuation-in-part of application No. 09/260,395, filed on Mar. 1, 1999, now Pat. No. 6,106,903.

(51) **Int. Cl.<sup>7</sup>** ..... **C23C 4/10**

(52) **U.S. Cl.** ..... **427/450**; 427/452; 264/80; 264/455

(58) **Field of Search** ..... 427/450, 452; 264/80, 455

(56) **References Cited**

**U.S. PATENT DOCUMENTS**

5,372,845 A \* 12/1994 Rangaswamy et al. .... 427/216  
5,454,999 A 10/1995 Jayashankar et al. .... 419/32

5,472,487 A \* 12/1995 Chin et al. .... 427/450

5,564,620 A \* 10/1996 Rawers et al. .... 228/265

6,106,903 A \* 8/2000 Upadhyā ..... 427/450  
6,110,853 A \* 8/2000 Berger et al. ..... 501/97.4

**OTHER PUBLICATIONS**

"Metals Handbook, Ninth Edition", American Society for Metals, vol. 5, pp. 363-365 and 374 (1982). (No month date).\*

J. Wolfenstine et al., Elevated-temperature mechanical behavior of plasma-sprayed MoSi<sub>2</sub>-SiC, *Materials Science and Engineering*, vol. A189, pp. 257-266 (1994) (No month date).

A.O. Kundrath et al., "Synthesis and application of composite TiC-Cr<sub>3</sub>C<sub>2</sub> targets," *Surface and Coatings Technology*, vol. 94-95, pp. 237-241 (1997). (No month date).

"Metals Handbook, Ninth Edition", American Society for Metals, vol. 5, pp. 363-365 and 374 (1982) (No month date).

\* cited by examiner

**Primary Examiner**—Katherine A. Bareford

(74) **Attorney, Agent, or Firm**—Gregory Garmong

(57) **ABSTRACT**

To prepare a thermally sprayed composite material, a pre-composited powder is first prepared and then thermally sprayed at an ambient pressure of no less than about 0.75 atmosphere in an oxidation-preventing atmosphere. The precomposed powder has a plurality of powder particles, and each powder particle is formed of a matrix and reinforcing particles distributed within and encapsulated by the matrix. The matrix has a composition of a matrix metal such as molybdenum, hafnium, zirconium titanium, vanadium, niobium, tantalum, or tungsten, and a matrix non-metal of silicon, boron, or carbon. The reinforcement particle is silicon carbide, boron carbide, silicon nitride, or boron nitride.

**20 Claims, 4 Drawing Sheets**





FIG. 1

FIG. 2  
FIG. 3





FIG. 6



100

FIG. 7

**THERMAL SPRAY FORMING OF A  
COMPOSITE MATERIAL HAVING A  
PARTICLE-REINFORCED MATRIX**

This application is a continuation-in-part of allowed application Ser. No. 09/260,395, filed Mar. 1, 1999, now U.S. Pat. No. 6,106,903, for which priority is claimed and whose disclosure is incorporated by reference.

This invention relates to the fabrication of composite materials, and, more particularly, to the fabrication of a particle-reinforced composite material by thermal spray processing.

**BACKGROUND OF THE INVENTION**

A number of metal silicides, boride, and carbides have great potential as coatings or freestanding structural materials for use in elevated-temperature applications. However, these materials typically exhibit a low fracture toughness at room temperature, low thermal shock resistance, and low creep resistance at elevated temperatures of greater than about 1100° C. These mechanical properties inhibit the utilization of the materials in otherwise attractive applications.

As discussed in the parent application Ser. No. 09/260,395, now U.S. Pat. No. 6,106,903, the mechanical properties of one of the members of this group, molybdenum disilicide, may be significantly improved by forming a composite material of particles of silicon carbide dispersed throughout the molybdenum disilicide. Such composite materials prepared by powder compaction and sintering techniques have exhibited improved room temperature toughness and elevated temperature strength. The presence of the silicon carbide also reduces the coefficient of thermal expansion of the composite material as compared with monolithic molybdenum disilicide. Powder techniques, however, are not practical for many applications, such as certain types of coatings and large freestanding structures.

Other fabrication techniques for composites of molybdenum disilicide and silicon carbide have been proposed. For example, U.S. Pat. No. 5,472,487 discloses the loose mixing of molybdenum disilicide and any of several other types of powders, silicon carbide being one of the disclosed other powders. This loose mixture of separated particles is applied by low pressure plasma spraying of the loose mixture. The present inventor has recognized that this disclosed approach may be well suited for the fabrication of some types of composite materials, but is of limited value in preparing a composite material containing silicon carbide, because of the elevated-temperature sublimation of silicon carbide from the solid state to the gaseous state during the low pressure plasma spraying. The sublimation of the silicon carbide results in its loss from the mixture, so that the amount of silicon carbide in the final product is substantially lower than in the starting material.

The parent application provided a solution to the problems associated with using the metal borides, silicides, and carbides in the specific case of molybdenum disilicide. There is a need to extend this solution to the more general case. The present invention fulfills this need, and further provides related advantages.

**SUMMARY OF THE INVENTION**

The present invention provides a method for preparing a particle-reinforced composite material. A wide range of volume fractions of reinforcement particles in the composite material may be prepared. Little if any of the reinforcement

material is lost in the deposition procedure, so that the final product has about the same volume fraction of reinforcement material as the starting material. The composite material is substantially fully dense, with few if any voids therein. The approach of the invention may be utilized to fabricate both coatings and freestanding structures. Large articles may be prepared relatively inexpensively, without the need for large containment chambers and the like.

In accordance with the invention, a method for preparing a mass of a thermally sprayed composite material comprises the steps of providing a precomposed powder comprising a plurality of powder particles, and thereafter thermal spray depositing the precomposed powder at an ambient pressure of no less than about 0.75 atmosphere in an oxidation-preventing atmosphere, to form a thermal sprayed mass.

Each powder particle comprises a matrix having a matrix composition comprising at least one matrix chemical combination of a matrix metal and a matrix non-metal selected from the group consisting of silicon, boron, and carbon, and mixtures thereof. Each powder particle further comprises a plurality of reinforcing particles, the reinforcing particles being distributed within and encapsulated by the relatively larger matrix and having a reinforcement-particle composition selected from the group consisting of silicon carbide, boron carbide, silicon nitride, and boron nitride.

The matrix metal is preferably selected from the group consisting of hafnium, zirconium titanium, vanadium, niobium, tantalum, and tungsten, and mixtures thereof. The preferred matrices prepared by this approach include silicides such as hafnium silicide, zirconium silicide, titanium silicide, vanadium silicide, niobium silicide, tantalum silicide, and tungsten silicide; borides such as hafnium boride, zirconium boride, titanium boride, vanadium boride, niobium boride, tantalum boride, and tungsten boride; and carbides such as hafnium carbide, zirconium carbide, titanium carbide, vanadium carbide, niobium carbide, tantalum carbide, and tungsten carbide.

The thermal sprayed mass typically comprises from about 5 volume percent to about 60 volume percent, more preferably from about 10 volume percent to about 50 volume percent, of the reinforcing particles, balance the matrix (plus any other constituents present).

The precomposed powder preferably comprises relatively finer reinforcement particles, preferably having a particle size of from about 0.1 micrometer to about 1 micrometer, distributed within and encapsulated by relatively coarser powder particles of the matrix composition, preferably having a particle size of from about 5 to about 80 micrometers. Such precomposed powder may be prepared using high temperature self-sustaining combustion synthesis or any other operable technique.

The thermal spraying is preferably accomplished by plasma spraying, most preferably argon-shrouded plasma spray deposition at 1 atmosphere ambient pressure. The thermal spraying may instead be accomplished in an environmental chamber with a protective atmosphere of argon or other oxidation-preventing gas. The argon-shrouded plasma spray approach is preferred because large areas or parts may be prepared without the expense of a correspondingly sized environmental chamber. The thermal spraying is typically accomplished by depositing the thermally sprayed precomposed powder onto a substrate, such as a surface to be coated or a form for a freestanding article. The thermal spray approach is relatively economical for fabricating large areas or structures.

After thermal spraying, the thermal sprayed mass may optionally be heat treated to stress relieve internal stresses

within the mass. Such internal stresses, where present and not relieved, may promote the premature failure of the thermal sprayed mass during thermal excursions or in other circumstances. The heat treatment is typically accomplished at a temperature of from about 800° C. to about 1400° C.

The present processing approach is carefully selected in order to fabricate the desired composite thermal sprayed mass. The precomposed powder must be used. The powder cannot be thermally sprayed as a loose mixture with separated particles of the matrix material and the reinforcement particles, as suggested by the '487 patent, because the reinforcement particles may sublime or otherwise degrade at elevated temperature. In that case where separated powders are used, a portion of the reinforcement may be lost as a vapor, and cannot be properly plasma sprayed because it is never present as a liquid phase that may bond with the matrix material. In the precomposed powder used in the present invention, the smaller, volatile reinforcement particles, and/or nitrides susceptible to decomposition such as silicon nitride, are encapsulated within the larger powder particles of the matrix phase, so that the liquification required for the successful thermal spraying is accomplished by the matrix material.

Further, the precomposed powder is applied by thermal spraying at about 0.75 atmosphere or greater ambient pressure, preferably at from about 0.75 atmosphere to about 1.25 atmospheres ambient pressure, and most preferably at 1 atmosphere ambient pressure. Spray fabrication of separated silicon carbide powder at greatly reduced pressures, as in the low-pressure plasma spray process used in the '487 patent, results in sublimation and at least partial evaporative loss of the silicon carbide. The combination of the use of precomposed powder and a spray process operating at about 0.75 atmospheres or greater pressure results in very little loss of the silicon carbide during application. Typically, the thermal sprayed mass has a volume percent of reinforcement particles that is no greater than 5 percentage points less than a volume percent of the reinforcement particles in the precomposed powder. For example, if the precomposed powder has about 45 volume percent of silicon carbide, the thermal sprayed mass would also have about 45 volume percent of silicon carbide, and in any event typically not less than about 40 volume percent of silicon carbide.

The avoidance of substantial loss of a volatile constituent during the thermal spraying operation is an important advantage of the present invention. Thermal sprayed composite masses with relatively large volume fractions of silicon carbide may be readily prepared. In reduced-pressure thermal spray processes using separated powders, by contrast, the maximum amount of a volatile constituent such as silicon carbide that may be incorporated in the final product is usually limited to less than about 10 volume percent due to the evaporation. Additionally, with the present approach it is not necessary to clean up substantial amounts of sublimed and evaporated silicon carbide from chamber walls, pumps, and the like as in the case of reduced-pressure spray processes.

Other features and advantages of the present invention will be apparent from the following more detailed description of the preferred embodiment, taken in conjunction with the accompanying drawings, which illustrate, by way of example, the principles of the invention. The scope of the invention is not, however, limited to this preferred embodiment.

#### BRIEF DESCRIPTION OF THE DRAWINGS

FIG. 1 is a block flow diagram of a preferred approach for practicing the present invention;

FIG. 2 is an idealized depiction of the microstructure of a precomposed powder of matrix particles and reinforcement particles;

5 FIG. 3 is an idealized depiction of the structure of a loose mixture of matrix-material particles and reinforcement particles that is not operable with the present invention;

FIG. 4 is a schematic view of a preferred apparatus for practicing the invention using a gas-shrouded plasma spray deposition torch;

10 FIG. 5 is an idealized depiction of a thermal sprayed mass prepared by the approach of the invention;

FIG. 6 is a schematic view of the apparatus of a second embodiment of the invention; and

15 FIG. 7 is a schematic view of an apparatus which is not in accordance with the invention.

#### DETAILED DESCRIPTION OF THE INVENTION

FIG. 1 depicts a preferred approach for preparing a mass 20 of composite material according to the invention. A precomposed powder of powder particles of a matrix composition with reinforcement particles embedded therein is provided, numeral 20. FIG. 2, which is not drawn to scale, illustrates several particles of such a precomposed powder 30. Finer 25 particles of the reinforcement material 32 are embedded within, distributed generally uniformly within, and encapsulated within a matrix of coarser powder particles 34. ("Finer" and "coarser" are used herein relative to each other, the finer particles being smaller than the coarser particles.) The powder particles 34 are preferably generally, but not necessarily exactly, equiaxed and nearly spherical. The reinforcement particles 32 are smaller than the powder particles 34, preferably much smaller. In a preferred form of the invention, the reinforcement particles 32 have a particle 30 size of from about 0.1 micrometer to about 1.0 micrometer (micron), more preferably from about 0.1 micrometer to about 0.5 micrometer, and the powder particles 34 a particle size of from about 5 micrometer to about 80 micrometers. Most preferably, the reinforcement particles 32 have a particle size of from about 0.1 micrometer to about 0.2 micrometers, and the powder particles 34 have a particle size of from about 70 micrometers to about 80 micrometers. That is, the reinforcement particles 32 preferably have sizes less than one percent of the sizes of the powder particles 34 in 40 which they are embedded and encapsulated. The reinforcement particles 32 are present in any operable volume fraction, but preferably in an amount of from about 5 volume percent to about 60 volume percent, more preferably from about 10 volume percent to about 50 volume percent, of the 45 total volume of the precomposed powder 30. An important feature of the present approach is that the reinforcement material of the reinforcement particles 32 is encapsulated within the powder particles 34, so that the reinforcement material cannot sublime and evaporate, or be oxidized or otherwise altered, during thermal spraying, and so that the 50 matrix composition of the powder particles 34 melts during thermal spraying to permit consolidation upon impingement upon a substrate.

The reinforcement particles 32 are silicon carbide, boron 60 carbide, silicon nitride, boron nitride, or mixtures thereof. ("Mixtures thereof" means in this context that any two or more of the listed types of particles may be mixed together.) These materials are selected because they are highly corrosion resistant and have high hardness. Their presence generally increases the toughness of the matrix materials which tend to be somewhat brittle and sometimes exhibit ductile-to-brittle transitions in lower temperature ranges.

The matrix in which the reinforcement particles **32** are embedded, which matrix material forms the balance of the powder particles **34**, has a matrix composition comprising at least one matrix chemical combination of a matrix metal, and a matrix non-metal selected from the group consisting of silicon, boron, and carbon, and mixtures thereof. The matrix metal is preferably selected from the group consisting of molybdenum, hafnium, zirconium, titanium, vanadium, niobium, tantalum, and tungsten, and mixtures thereof. Thus, in the three main embodiments of the matrix material, the matrix material is selected from the group consisting of molybdenum silicide, hafnium silicide, zirconium silicide, titanium silicide, vanadium silicide, niobium silicide, tantalum silicide, and tungsten silicide; selected from the group consisting of hafnium boride, zirconium boride, titanium boride, vanadium boride, niobium boride, tantalum boride, and tungsten boride; or selected from the group consisting of molybdenum carbide, hafnium carbide, zirconium carbide, titanium carbide, vanadium carbide, niobium carbide, tantalum carbide, and tungsten carbide. (As used herein, the generic term encompasses available chemical variations. For example, "molybdenum silicide" includes, but is not limited to, molybdenum disilicide.) Mixtures may be formed from within or between these various groups. For example, some of the powder particles **34** may have a hafnium boride ( $HfB_2$ ) matrix with boron carbide reinforcement particles, and some of the powder particles may have a molybdenum silicide matrix with silicon carbide reinforcement particles.

The precomposed powder is made by any operable approach. Preferably, it is prepared by high temperature self-sustaining combustion synthesis, a known process which is described, for example, in U.S. Pat. Nos. 4,402,776 and 5,564,620, and in A. O. Kunrath et al., "Synthesis and application of composite TiC— $Cr_3C_2$  targets", *Surface and Coatings Technology*, vol. 94–95 (1997), pages 237–241.

FIG. 3 illustrates a form of separated powder mixture **36** which is not operable in the invention and is not within the scope of the term "precomposed powder" as used herein. In this separated powder mixture **36**, particles **38** of some potential reinforcing material **38** and particles **40** of some potential matrix material are loose and separated from each other. The particles **38** are not embedded within, distributed generally uniformly within, or encapsulated within the particles **40**.

Returning to FIG. 1, the precomposed powder is thermal sprayed, numeral **22**, to form a thermal sprayed mass. Any operable thermal spray approach may be used, as long as it is conducted at an ambient pressure of no less than about 0.75 atmosphere (1 atmosphere is approximately 14.7 pounds per square inch) and in an oxidation-preventing, nonreactive atmosphere to prevent oxidation of the thermally sprayed material and the substrate being sprayed. The "ambient" pressure is that externally surrounding the powder as it is thermally sprayed.

A preferred thermal spray apparatus is illustrated in FIG. 4. An argon-shrouded plasma spray deposition apparatus **50** includes a central electrode **52** that is electrically negatively biased with respect to a concentric tubular body **54** of the apparatus **50**. Electrons **56** are emitted from the central electrode **52** into the interior of the tubular body **54**. Precomposed powder **30**, as described above, and optionally an inert, non-oxidizing, fluidizing gas such as argon, are supplied through an input tube **58** and flowed through the tubular body **54**. Additional inert, non-oxidizing gas, preferably argon, may optionally be flowed through the tubular body **54** through an argon input **59**. In operation, an electrical arc **60** is struck between the apparatus **50** and a target

substrate **61**, forming a plasma. At least a portion of the matrix material of the powder particles **34** at the surface of the precomposed powder **30** is melted as the precomposed powder **30** flows through the electrical arc **60** and associated plasma and toward the substrate **61**. Upon striking the substrate **61**, or previously deposited material **62** overlying the substrate **61**, the melted portion of the precomposed powder **30** solidifies to form a thermal sprayed mass **64**. The reinforcement powder encapsulated within the matrix material of the powder particles **34** need not melt to a liquid phase, as is required in conventional plasma spray deposition. The reinforcement particles **32** cannot be evaporatively lost, because they are encapsulated within the powder particles **34**.

10 A concentric shroud tube **66** surrounds and overlies the powder tube **56**. A nonreactive gas that prevents oxidation, such as an inert gas and most preferably argon, is flowed through an argon input **67** and thence through the shroud tube **66**, and exits to form a gas shroud **68** surrounding the electrical arc **60** and plasma, and the partially melted precomposed powder **30** therein. The gas shroud **68** also extends over the most recently deposited thermal sprayed mass **64**. The gas shroud **68** prevents oxidation of the partially melted precomposed powder **30** and the most recently deposited thermal sprayed mass **64**, allowing it to cool to a sufficiently low temperature that oxidation is no longer a concern. (Other nonreactive gases such as helium or nitrogen may be used.)

15 The plasma spray deposition apparatus **50** is operated in the ambient atmosphere without any vacuum chamber or environmental control chamber, most preferably at one atmosphere ambient pressure. It therefore may be moved freely about, to be used to form either relatively thin coatings on the substrate or relatively thick layers that are 20 freestanding, regardless of the size of the substrate. One significant limitation of many other spray deposition procedures is that they must be operated in vacuum chambers or other types of environmental control chambers, effectively limiting the size and configuration of the substrate unless 25 very large and expensive chambers are available. The present apparatus may also be used for on-site repairs, which is often not possible for those techniques requiring environmental control chambers.

30 FIG. 5 illustrates the resulting structure of the thermal sprayed mass **64**. The thermal sprayed mass **64** is formed of the resolidified particles **70** of precomposed powder **30**, which have been partially melted on their outer surfaces, forced together at impact upon their target, and resolidified in a dense, mass having few, if any, voids or pores therein. 35 The thermal sprayed mass **64** is formed of the reinforcement particles **32** distributed generally uniformly within the reshaped powder particles **34**. The resolidified particles **70** are typically flattened in the direction perpendicular to the direction of thermal spray deposition onto the substrate **61** 40 (from the top toward the bottom in FIG. 5). An important feature of the invention is that during the thermal spray deposition the reinforcement particles **32** are never exposed to vacuum or to the ambient environment, because they are 45 encapsulated within the matrix material of the powder particles **34**. Consequently, very little, if any, reinforcement material of the reinforcement particles **32** is lost to sublimation and/or evaporation, or is chemically changed as by 50 oxidation or other reaction, so that the volume fraction of reinforcement material in the solidified thermal sprayed mass **64** is the same or substantially the same as that in the starting material, the precomposed powder **30**. At most, 55 there would be reduction in volume fraction of the rein-

forcement material of the powder particles 32 of 5 percent-  
age points from the precomposed powder 30 to the thermal  
sprayed mass 64, but in practice that figure is much nearer  
to zero loss of reinforcement material.

An important feature of the preferred embodiment is that  
it requires no environmental control chamber. In some cases,  
providing a controlled environment may not be difficult, and  
the present invention may be used in conjunction with an  
environmental control chamber. In the second embodiment  
illustrated in FIG. 6, an environmental control chamber 80  
is used to produce a protective environment at an ambient  
pressure of about 0.75 atmospheres or greater. In the illus-  
trated case, argon or other non-oxidizing, non-reactive gas  
flows through the environmental control chamber to estab-  
lish the protective atmosphere. The thermal spray may be  
produced with an electrical arc, as in the plasma spray  
deposition apparatus 50, but an alternative approach is  
illustrated in FIG. 6. Here, a combustion gas and oxidizer  
(for example, hydrogen and oxygen) are supplied and  
flowed through a central tube 82. The combustion gas and  
oxidizer are ignited to form a plasma 84. Precomposed  
powder and argon gas are flowed through an outer tube 86  
and into the plasma. The outer surface of the precomposed  
powder 30 is partially melted in the plasma and deposited  
upon the substrate 61 as the thermal sprayed mass 64, as  
described previously. No shroud gas is required, inasmuch  
as the entire interior of the environmental control chamber  
is filled with the non-oxidizing, non-reactive gas. Other  
techniques for forming the plasma, such as laser energy, may  
be used.

Returning to FIG. 1, the as-deposited thermal sprayed  
mass may optionally be heat treated, numeral 24. The heat  
treatment is performed to relieve internal stresses in the  
thermal sprayed mass. A preferred heat treatment is to heat  
the thermal sprayed mass 64 to a temperature of from about  
800° C. to about 1400° C., more preferably from about 800°  
C. to about 1000° C., for a time of from about 30 minutes  
to about 5 hours, in an inert gas such as argon. The heat  
treatment also allows the crystal structure of the matrix  
material to be established uniformly as a more nearly  
equiaxed crystalline phase with the flattened grains illus-  
trated in FIG. 5.

FIG. 7 illustrates an approach which is not within the  
scope of the present invention. In this deposition apparatus  
100, a chamber 102 is evacuated to a sub-atmospheric  
pressure below about 0.75 atmosphere, typically about 0.25  
atmosphere or less. A plasma 104 is formed between an  
electrode 106 and a substrate 108. The plasma may be  
formed by combustion or other approach as well. The matrix  
material and the reinforcement particles, both fluidized in a  
gas such as argon, are furnished in a loose, separated form,  
as was illustrated in FIG. 3. That is, the matrix material and  
the reinforcement particles are not precomposed. The  
matrix material and the reinforcement particles are flowed  
into a powder tube 110, where they mix and flow into the  
plasma 104, where the matrix material at least partially  
melts. The reinforcement material, however, typically does  
not melt, but instead sublimes, evaporates, or chemically  
reacts, at least in part. There is a large loss of the reinforce-  
ment material to evaporation, which evaporated material  
coats the interior of the chamber 102 or is drawn into the  
vacuum system where it must be cleaned out. The volume  
fraction of reinforcement in the final deposit is substantially  
less than the associated ratio in the starting powders. It may  
be expected that the volume fraction of reinforcement mate-  
rial may be limited to no more than about 10 volume percent  
in some cases due to sublimation, which may be too low for

many applications. In one case using this approach that is  
not within the scope of the present invention, it was reported  
that the silicon carbide was 20 volume percent of the total of  
the starting feed mass of molybdenum disilicide and silicon  
carbide, but was present in an amount of only 9 percent of  
the deposit on the substrate.

The present invention has been reduced to practice with  
the argon-shrouded plasma spray apparatus of FIG. 4. Coat-  
ings were produced on a silicon carbide foam substrate in  
thicknesses of 0.012, 0.016, 0.017, 0.018, 0.022, and 0.030  
inches. Final thermal sprayed masses were produced with  
nominal silicon carbide contents of 25, 35, and 45 volume  
percent. (Molybdenum disilicide coatings with no silicon  
carbide present were produced as controls.) The specimen  
with a nominal silicon carbide content of 45 volume percent  
had 45 volume percent of silicon carbide in the precompos-  
ited powder 30 feed material. This specimen was measured  
by image microanalysis techniques to have between 44 and  
46 volume percent of silicon carbide in the deposited  
thermal sprayed mass. That is, within the experimental error  
of the measurements, no silicon carbide was lost from the  
precomposed powder during the argon shrouded plasma  
deposition.

Various of the specimens were tested to determine rel-  
25 evant mechanical and physical properties. Molybdenum  
disilicide with 25 volume percent of silicon carbide in a  
thickness of 0.017 inches, molybdenum disilicide with 25  
volume percent of silicon carbide in a thickness of 0.018  
inches, molybdenum disilicide with 25 volume percent of  
30 silicon carbide in a thickness of 0.025 inches, molybdenum  
disilicide with 45 volume percent of silicon carbide in a  
thickness of 0.018 inches, and molybdenum disilicide with  
45 volume percent of silicon carbide in a thickness of 0.025  
inches exhibited no cracking or spallation when heated to  
35 1500° C. in an inert atmosphere, to evaluate mechanical  
properties. The molybdenum disilicide coatings with no  
silicon carbide present exhibited cracking and spallation in  
this same test.

In an oxidation test, molybdenum disilicide with 25  
volume percent of silicon carbide in a thickness of 0.016  
inches thick and molybdenum disilicide with 45 volume  
percent of silicon carbide in a thickness of 0.025 inches were  
40 heated in air with an oxyacetylene torch to 1600–1700° C.  
The specimens exhibited no oxidation damage. Specimens  
of the other coatings were tested to 1500–1600° C. in a  
similar manner, and showed no oxidation damage.

In another reduction to practice, a coating was prepared  
with about 55 percent by volume of silicon carbide particles  
50 in a matrix of hafnium boride.

Although a particular embodiment of the invention has  
been described in detail for purposes of illustration, various  
modifications and enhancements may be made without  
departing from the spirit and scope of the invention.  
55 Accordingly, the invention is not to be limited except as by  
the appended claims.

What is claimed is:

1. A method for preparing a mass of a thermally sprayed  
composite material, comprising the steps of  
60 providing a precomposed powder comprising a plurality  
of powder particles, each powder particle consisting of  
a matrix having a matrix composition comprising at  
least one matrix chemical combination of  
a matrix metal, and  
65 a matrix non-metal selected from the group consist-  
ing of silicon, boron, and carbon, and mixtures  
thereof, and

a plurality of reinforcing particles, the reinforcing particles being distributed within and encapsulated by the relatively larger matrix and having a reinforcement-particle composition selected from the group consisting of silicon carbide, boron carbide, boron nitride, and mixtures thereof; and thereafter

10 thermal spray depositing the precomposed powder at an ambient pressure of no less than about 0.75 atmosphere in an oxidation-preventing atmosphere, to form a thermal sprayed mass.

15 2. The method of claim 1, wherein the precomposed powder comprises the reinforcing particles having a reinforcing-particle size of from about 0.1 micrometer to about 1.0 micrometer, distributed within the powder particles having a particle size of from about 5 micrometers to about 80 micrometers.

20 3. The method of claim 1, wherein the step of providing a mixture includes the step of

25 preparing the precomposed powder using high temperature self-sustaining combustion synthesis.

30 4. The method of claim 1, wherein the oxidation-preventing atmosphere is an argon atmosphere.

35 5. The method of claim 1, wherein the step of thermal spray depositing includes the step of

40 thermal spray depositing the precomposed powder by argon-shrouded plasma spray deposition.

45 6. The method of claim 1, wherein the step of thermal spray depositing is performed at 1 atmosphere ambient pressure.

50 7. The method of claim 1, wherein the step of thermal spray depositing is performed at an ambient pressure of from about 0.75 atmosphere to about 1.25 atmosphere.

55 8. The method of claim 1, wherein the step of thermal spray depositing is performed in an environmental chamber.

60 9. The method of claim 1, wherein the step of thermal spray depositing includes the step of

65 thermal spray depositing the precomposed powder onto a substrate.

70 10. The method of claim 1, wherein the thermal sprayed mass is a coating.

75 11. The method of claim 1, wherein the thermal sprayed mass is a freestanding structure.

80 12. The method of claim 1, wherein the thermal sprayed mass comprises from about 5 volume percent of the reinforcing particles to about 60 volume percent of the reinforcing particles, balance matrix composition.

85 13. The method of claim 1, wherein the thermal sprayed mass comprises a volume percent of the reinforcing particles that is no greater than 5 percentage points less than a volume percent of the reinforcing particles in the precomposed powder.

90 14. A method for preparing a mass of a thermally sprayed composites material, comprising the steps of

95 providing a precomposed powder comprising a plurality of powder particles, each powder particle consisting of a matrix having a matrix composition comprising at least one matrix chemical combination of a matrix metal, and a matrix non-metal selected from the group consisting of silicon, boron, and carbon, and mixtures thereof, and

a plurality of reinforcing particles, the reinforcing particles being distributed within and encapsulated by the relatively larger matrix and having a reinforcement-particle composition selected from the group consisting of silicon carbide, boron carbide, silicon nitride, boron nitride, and mixtures thereof; and thereafter

100 thermal spray depositing the precomposed powder at an ambient pressure of no less than about 0.75 atmosphere in an oxidation-preventing atmosphere, to form a thermal sprayed mass; and thereafter heat treating the thermal sprayed mass.

105 15. The method of claim 14, wherein the step of heat treating includes the step of heating the thermal sprayed mass to a temperature sufficient to relieve internal stresses therein.

110 16. The method of claim 14, wherein the step of heat treating includes the step of heating the thermal sprayed mass to a temperature of from about 800° C. to about 1400° C.

115 17. A method for preparing a mass of a thermally sprayed composite material, comprising the steps of

120 providing a precomposed powder comprising a plurality of powder particles, each powder particle having a matrix having a composition consisting of at least one matrix chemical combination of a matrix metal selected from the group consisting of molybdenum, hafnium, zirconium, titanium, vanadium, niobium, tantalum, and tungsten, and mixtures thereof, and

125 a matrix non-metal selected from the group consisting of silicon, boron, and carbon, and mixtures thereof, and

130 a plurality of reinforcing particles, the reinforcing particles being distributed within and encapsulated by the relatively larger matrix and having a reinforcement-particle composition selected from the group consisting of silicon carbide, boron carbide, silicon nitride, boron nitride, and mixtures thereof, the matrix forming the balance of each powder particle, the matrix forming the balance of each powder particle; and thereafter

135 thermal spray depositing the precomposed powder at an ambient pressure of no less than about 0.75 atmosphere in an oxidation-preventing atmosphere, to form a thermal sprayed mass.

140 18. The method of claim 17, wherein the precomposed powder comprises a matrix composition selected from the group consisting of molybdenum silicide, hafnium silicide, zirconium silicide, titanium silicide, vanadium silicide, niobium silicide, tantalum silicide, and tungsten silicide.

145 19. The method of claim 17, wherein the precomposed powder comprises a matrix composition selected from the group consisting of hafnium boride, zirconium boride, titanium boride, vanadium boride, niobium boride, tantalum boride, and tungsten boride.

150 20. The method of claim 17, wherein the precomposed powder comprises a matrix composition selected from the group consisting of molybdenum carbide, hafnium carbide, zirconium carbide, titanium carbide, vanadium carbide, niobium carbide, tantalum carbide, and tungsten carbide.